

Dec. 24, 1963

P. ZOURAEFF ET AL

3,115,249

EXTRUSION SYSTEM

Filed July 7, 1958

2 Sheets-Sheet 1



INVENTORS

PETER ZOURAEFF  
ANDREW G. FORREST

by their attorneys  
*Glenn and Jackson*

Dec. 24, 1963

P. ZOURAEFF ET AL.

3,115,249

EXTRUSION SYSTEM

Filed July 7, 1958

2 Sheets-Sheet 2



INVENTORS  
PETER ZOURAEFF  
ANDREW G. FORREST

by their attorneys  
Glenn and Jackson

1

3,115,249

## EXTRUSION SYSTEM

Peter Zouraeff, Phoenix, Ariz., and Andrew G. Forrest, Richmond, Va., assignors to Reynolds Metals Company, Richmond, Va., a corporation of Delaware

Filed July 7, 1958, Ser. No. 746,926

2 Claims. (Cl. 207—10)

This invention relates to means and method of extruding plain carbon, alloy and stainless steels, titanium, titanium alloy and other high temperature materials, and is a continuation-in-part of application Serial No. 655,662, filed April 29, 1957, for Titanium Extrusion System, now abandoned.

Various methods of extruding the subject metals have been used, but the products of these extrusion methods have been found to have surface blemishes, and other imperfections, such as laps, seams, cracks and/or porous conditions, such that it has been found necessary to produce the extrusions in sizes about  $\frac{1}{16}$  of an inch thicker on all outside surfaces than specified final dimensions. The excess thickness is then machined and ground down to size, which is an expensive operation.

It is a primary object of the invention to eliminate the disadvantages of prior extrusion methods.

It is a further object to extrude materials in sections having higher quality finishes than formerly possible. By use of the method of this invention, extrusions having surface roughnesses as low as 10 microinches arithmetic average have been produced.

Another object of the invention is to extrude shapes of smaller cross section than can be made by conventional means from the same size tooling.

Still another object is to extrude thinner sections than can be produced by conventional methods from the same size tooling.

A further object is to extrude shapes held to closer tolerances than those produced by other methods.

Yet a further object is to provide an extrusion method which will materially lessen the cost of fabricating high temperature materials.

In accordance with the present invention, the subject metals can be extruded with such improved quality of product that the cross-sectional shape of the extrusion can be made equal, within commercial practice tolerances, to the specified final dimensions, in such cases, for example, as parts for air frames. In the case of some jet engine parts, special design considerations may require some subsequent machining, but even in that case the amount of such machining is substantially reduced as compared to extrusions by present conventional methods. In addition, the extrusion system of the invention enables thinner web sections to be extruded than are possible by conventional methods. Similarly, extrusions of smaller cross-sectional areas can be produced than are possible by conventional methods with comparable equipment.

The improved results of the invention are obtained by observing the following concurrent limitations regarding (1) the extrusion die, (2) the extrusion lubricant, and (3) the extrusion operating conditions of speed, billet temperature and extrusion ratio:

(1) *Extrusion die*.—The die must be sloped and contoured on its inner face against which the billet is squeezed, in order to squeeze the billet progressively down to the size of the die slot as the billet metal approaches the slot. The design of each die must be adapted to the shape of the particular slot, according to known practices of die contouring, for the purpose of avoiding any shearing action such as would result from use of a flat-faced die. One aspect of the avoidance of shearing action is the avoidance of "dead pockets" of billet metal which

2

become detached from the main body of metal moving toward the slot, but may subsequently be carried through the slot, and weaken the extrusion because of the tendency of the pocket to become detached from the main body of the extrusion. The pockets also tend to corrugate and thereby cause laps in the metal which passes over the dead pocket on its way toward the die slot.

The dies may be either machined from forged blanks or cast directly to the desired configuration. In order to prolong the working life of the die, it is preferred that its bearing surfaces are of a chrome-cobalt alloy or like hard alloy. In the case of a cast die, this material may be cast directly into the bearing configuration. Since the machining of whole blanks of these hard alloys is very difficult and costly, it is preferred in this practice in the case of machined die that the hard alloy be applied by welding to the bearing areas and then machined or ground to final size. In order to produce complex shapes, it is the preferred practice in accordance with the invention to use a "split die" made up of different sections which are made separately and then assembled to form the complete die.

The accompanying drawings illustrate a present preferred example of a die used in accordance with the invention, as hereinafter more particularly described.

(2) *Extrusion lubricant*.—A thin layer of micaceous particles disposed against the contoured faces of the die is necessary to lubricate the said faces as they squeeze down the billet, in order to prevent galling of the metal as it is forced through the die. The micaceous particles preferably have a particle size of about one micron, and are capable of internal shearing of the particles to provide the necessary lubricating action under the elevated temperatures and pressures within the die during the extrusion operation. The present preferred example of the micaceous lubricant is biotite, and other examples are muscovite and vermiculite. It is necessary to adhere the layer of micaceous particles to the walls of the die in such manner as to insure that they will be there when the preheated billet is compressed against the die walls, and for that purpose the said particles are admixed with an adherent binding agent, the present preferred example of which is a grease formed of a heavy petroleum oil gelled with bentonite clay. This grease has the ability of holding the layer of micaceous particles against the die walls in spite of the tendency of the grease to volatilize when the preheated billet is placed in the die cavity.

Examples of the lubricant and binder of the invention are hereinafter specified with greater particularity.

(3) *Extrusion conditions*.—(a) *Speed of extrusion*.—The speed of extrusion in terms of movement of the extruded part from the die is approximately constant during the extrusion operation, and for the purposes of the invention the average speed of extrusion during the extrusion operation is in the range of about 40 to about 350 feet per minute, and is preferably about 180 feet per minute. Higher extrusion speeds require excessive power and correspondingly powerful and expensive equipment, and lower speeds take too much time and introduce problems resulting from dissipation of heat during prolonged periods of extrusion.

(b) *Extrusion ratio*.—The extrusion ratio is the ratio of the cross-sectional area of the cylinder within which the billet is placed for extrusion, to the cross-sectional area of the die slot, and, for the purposes of the invention, is in the range of about 10/1 to about 50/1. Higher extrusion ratios require excessive power, and lower extrusion ratios are apt to fail to work the metal sufficiently to produce a satisfactory extruded product. In general, an extrusion ratio in the range of about 15/1 to about 25/1 is preferred.

(c) *Billet temperature*.—The temperature of the billet

when the extrusion operation begins must, for the purposes of the invention, be in the range of about 1300° F. to about 2400° F., depending on the nature of the particular subject metal being extruded, and the temperature rise before the metal passes out of the die slot, which is governed by such factors as the rate of extrusion and other extrusion conditions.

For a better understanding of the invention, reference is made to the present preferred embodiment thereof shown, for purposes of illustration only, in the accompanying drawings. In the drawings:

FIG. 1 is a cross-sectional view taken vertically through the central axis of an extrusion press and showing the extrusion of a subject metal billet, in accordance with the invention;

FIG. 2 is an end view in elevation of the extrusion die shown in FIG. 1, showing the face of the die against which the billet is pressed;

FIGS. 3, 4 and 5 are enlarged, fragmentary, cross-sectional views taken on the lines 3-3, 4-4 and 5-5, respectively, of FIG. 2, and

FIG. 6 is an enlarged side view in elevation taken on the line 6-6 in FIG. 2 and showing the face of one of the two split portions of the die shown in FIG. 1.

Referring now more particularly to the drawings, FIG. 1 shows an extrusion press 10 in which a subject metal billet 12 in the liner 15 of a container 14 is being compressed by a ram 16 and dummy block 18 and extruded through a die 20 to form an elongated extrusion 22. The die 20 is removably mounted in a certain die holder 24 and conventional supporting elements hold the die against axial thrust. Conventional resistance heater elements (not shown) are provided to preheat the liner, and the die is readily removable and replaceable to facilitate cleaning and preheating the die before each extrusion operation.

The die 20 is of split construction to facilitate constructing the die to produce sections such as the I section

of the illustrated extrusion 22. In accordance with present preferred practice, the die slot 26 is centered in the middle of the die, and is bisected by the split of the die, preferably along the plane of symmetry of the slot, where 5 the slot is symmetrical, as illustrated. The face of the die along which the billet metal flows toward the slot has a generally conical depression 28 sloping from the outer periphery of the die toward the slot, in order to guide the metal toward the slot in such a way as to avoid any shearing of the metal. The initial lead-in slope changes 10 near the slot, in smoothly contoured curves 30 which are tangent to the lead-in slope 28 and to the final bearing walls 32 of the slot. The metal is thus channeled smoothly along the inside face of the die until it passes 15 out through the slot 26.

Before the billet is inserted in the container, a thin and substantially uniform layer of the lubricant of the invention is swabbed around the interior surface of the container which will be in contact with the billet. Likewise, 20 before the die is replaced on the container at the beginning of an extrusion operation, all of the die surfaces which will be in contact with the billet are similarly coated. A present preferred example of the lubricant is a mixture of equal proportions of biotite, having a particle size of one micron or less, and an adherent carrier consisting of petroleum oil mixed with enough bentonite clay to give it the consistency of a light grease (such a carrier, known as a bentone grease, is commercially available as "Fiske #525" of Fiske Brothers Refining Company, Newark, N.J.). If higher proportions of biotite are used, or if other methods of application are substituted, such as spraying, the viscosity of the carrier may have to be altered by thinning with more volatile petroleum oils or the like. Ranges of proportions of from 25% to 75% by weight of biotite, the balance being "Fiske #525," can be used, and a wider range is possible, but not preferred.

Further details of the practice of the invention are illustrated in the following table of examples:

Table of Examples

| Material                                                         | Billet Preheat, ° F. | Extrusion Ratio | Extrusion Speed, ft./min. | Product                              |
|------------------------------------------------------------------|----------------------|-----------------|---------------------------|--------------------------------------|
| I. Plain Carbon Steels: Example 1—<br>SAE 1020 Steel.            | 2,400                | 32:1            | 350                       | 1" round.                            |
| II. Alloy Steels:                                                |                      |                 |                           |                                      |
| Example 2—SAE 4340 Steel                                         | 2,400                | 32:1            | 350                       | T section—.125" thickness.           |
| Example 3—SAE 4130 Steel                                         | 2,400                | 32:1            | 350                       | Do.                                  |
| III. Stainless Steels:                                           |                      |                 |                           |                                      |
| Example 4—422M                                                   | 2,400                | 32:1            | 340                       | Do.                                  |
| Example 5—PH17-4                                                 | 2,400                | 32:1            | 320                       | Do.                                  |
| Example 6—PH17-7                                                 | 2,400                | 18:1            | 270                       | L section—.250" and .125".           |
| IV. Hot Work Tool Steels:                                        |                      |                 |                           |                                      |
| Example 7—Vaser Jet 1000                                         | 1,950                | 13:1            | 320                       | H beam—.150" thickness.              |
| Example 8—Peerless 56 (66S)                                      | 2,000                | 23:1            | 286                       | I beam—.125" thickness.              |
| V. Special Hi-Temp Metals: Example 9—A286 (25% Ni-15% Cr).       | 2,100                | 14:1            | 168                       | Angle—.300" thickness.               |
| VI. Commercially pure titanium:                                  |                      |                 |                           |                                      |
| Example 10                                                       | 1,650                | 21:1            | 80                        | Engine Sections:                     |
| Example 11                                                       | 1,700                | 32:1            | 120                       | 10 ft. x 1.5 sq. in.                 |
| Example 12                                                       | 1,550                | 16:1            | 60                        | 14 ft. x 1 sq. in.                   |
|                                                                  |                      |                 |                           | 8 ft. x 2 sq. in.                    |
| VII. Alpha-beta titanium alloys:                                 |                      |                 |                           |                                      |
| (a) 6% Al, 4% V, bal. Ti—                                        |                      |                 |                           | I-beams:                             |
| Example 13                                                       | 1,650                | 26:1            | 140                       | 8 ft. x 0.7 sq. in.                  |
| Example 14                                                       | 1,800                | 26:1            | 80                        | 8 ft. x 0.7 sq. in.                  |
| Example 15                                                       | 1,750                | 21:1            | 120                       | 8 ft. x 0.7 sq. in.                  |
| Example 16                                                       | 1,650                | 21:1            | 240                       | Engine Section, 10 ft. x 1.5 sq. in. |
| (b) 4% Al, 4% Mn, bal. Ti—                                       |                      |                 |                           | I-beam, 8 ft. x 0.7 sq. in.          |
| Example 17                                                       | 1,700                | 26:1            | 225                       | Engine Section, 10 ft. x 1.5 sq. in. |
| Example 18                                                       | 1,650                | 21:1            | 120                       |                                      |
| (c) 3% Al, 5% Cr, bal. Ti—                                       |                      |                 |                           | I-beam, 8 ft. x 0.7 sq. in.          |
| Example 19                                                       | 1,700                | 26:1            | 225                       | Engine Section, 10 ft. x 1.5 sq. in. |
| Example 20                                                       | 1,650                | 21:1            | 120                       |                                      |
| (d) 3% Mn, 1% Cr, 1% Fe and Mo, 1% V, bal. Ti—                   |                      |                 |                           |                                      |
| Example 21                                                       | 1,650                | 20:1            | 60                        |                                      |
| VIII. Alpha Titanium alloys: 5% Al, 2.5% Sn, bal. Ti—Example 22. | 1,850                | 34:1            | 305                       | Engine Section, 10 ft. x 1.5 sq. in. |
|                                                                  |                      |                 |                           | T-Section, 8 ft. x 0.4 sq. in.       |

In Examples 1-9 of the above table the various steel samples are commercially well known and are comprised of iron containing other metals alloyed therewith in approximately the nominal percentages by weight as shown in the following tabulation:

|                         | SAE-1020 | SAE-4130 | SAE-4340 | PH-17-4 | PH-17-7 | Vasco Jet 1000 | Peerless 56 | 422-M | A-286 |
|-------------------------|----------|----------|----------|---------|---------|----------------|-------------|-------|-------|
| Carbon                  | .20      | .30      | .40      | 1.07    | 1.09    | .35            | .40         | .28   | .05   |
| Chromium                | .95      |          | .80      | 17.0    | 17.0    | 5.0            | 3.3         | 12.0  |       |
| Nickel                  |          |          | 1.75     | 4.0     | 7.0     |                |             | .20   | 26.0  |
| Copper                  |          |          |          | 4.0     |         |                |             |       |       |
| Manganese               | .45      | .50      | .70      | 1.1.0   | 1.1.0   | .35            | .60         | .84   | 1.35  |
| Silicon                 |          | .30      | .30      |         |         | .90            | 1.0         | .25   | .35   |
| Molybdenum              |          | .20      | .25      |         |         | 1.3            | 2.75        | 2.25  | 1.75  |
| Aluminum                |          |          |          |         | 1.0     |                |             |       | .20   |
| Phosphorous             | 1.04     | 1.04     | 1.04     |         |         |                |             |       |       |
| Vanadium                |          |          |          |         |         | .45            | .40         | .50   | .30   |
| Tungsten                |          |          |          |         |         |                |             | 1.70  |       |
| Titanium                |          |          |          |         |         |                |             |       | 2.0   |
| Columbium plus Tantalum |          |          |          |         |         |                |             |       |       |
| Sulfur                  | 1.05     | 1.04     | 1.04     |         | .30     |                |             |       |       |

<sup>1</sup> Denotes maximum limit.

Above are iron base alloys.

The products identified in the above table have an excellent finish and have dimensions within commercial practice tolerances, so that subsequent machining is unnecessary in the case of air frame sections, for example, and in the case of engine sections is necessary only to a limited extent due to the special requirements of subsequent fabricating operations on engine sections. The extrusions possess an internal structure capable of satisfactory heat-treatment response in the case of certain alloys when produced within temperature limits suitable for that purpose during extrusion; e.g., Examples 5 and 6. In order to take full advantage of billet preheating, and to obtain the best results, the container and die are preferably preheated before the extrusion operation. The container is preferably preheated to about 800 to 900° F. Typical die preheat temperatures for the operations shown in the above table are in the range 400 to 1050° F.

While we have illustrated and described certain present preferred examples of the invention and methods of practicing the same, it will be recognized that the invention may be otherwise variously embodied and practiced within the scope of the following claims.

What is claimed and desired to be secured by Letters Patent is:

1. The method of extruding high temperature metals selected from the group consisting of plain carbon, alloy and stainless steels, titanium and titanium alloys, substantially directly to final dimensions with the surface thereof characterized by the absence of blemishes and having an average surface roughness as low as 10 microinches, which comprises the steps of preheating a billet of the aforesaid metal to a temperature in the range of 1300° F. to about 2400° F., placing said billet next to an extrusion die having a sloped, contoured inner face and provided with an extrusion opening of a size and shape to form the billet substantially exactly to the final dimensions desired, the opening having a cross-sectional area within the range of about  $\frac{1}{10}$  to about  $\frac{1}{5}$  of the cross-sectional area of the billet, coating the surfaces of the die which en-

gage the billet during extrusion with a lubricant consisting of micaceous particles carried in an adherent grease with the micaceous particles being not more than one micron in size and constituting at least 25% by weight of said lubricant, and compressing the billet against the

die to extrude the metal through said extrusion opening 25 of the die at an average rate in the range of about 40 to about 350 feet per minute.

2. The method according to claim 1 in which the micaceous particles are selected from the group consisting of biotite, vermiculite and muscovite, and the adherent grease 30 is a petroleum grease gelled with bentonite clay, said micaceous particles being in the range of from about 25% to about 75% by weight of the lubricant.

#### References Cited in the file of this patent

#### UNITED STATES PATENTS

|    |           |                |                |
|----|-----------|----------------|----------------|
| 35 | 140,567   | York           | July 1, 1873   |
|    | 1,066,971 | Adams          | July 8, 1913   |
|    | 2,063,563 | Sparks         | Dec. 8, 1936   |
| 40 | 2,322,738 | Rouse          | June 22, 1943  |
|    | 2,623,852 | Peterson       | Dec. 30, 1952  |
|    | 2,731,145 | Kritscher      | Jan. 17, 1956  |
|    | 2,735,814 | Hodson et al.  | Feb. 21, 1956  |
| 45 | 2,753,261 | Goetzel et al. | July 3, 1956   |
|    | 2,757,794 | Walgren        | Aug. 7, 1956   |
|    | 2,806,596 | Dodds et al.   | Sept. 17, 1957 |
|    | 2,821,475 | Jaffee et al.  | Jan. 28, 1958  |
|    | 2,832,468 | Krause         | Apr. 29, 1958  |
| 50 | 2,837,425 | Vordahl        | June 3, 1958   |

#### FOREIGN PATENTS

|         |               |               |
|---------|---------------|---------------|
| 726,917 | Great Britain | Mar. 23, 1955 |
|---------|---------------|---------------|

#### OTHER REFERENCES

- 55 "Metal Flow and the Extrusion Defect," pp. 108-112, American Machinist, May 15, 1950.  
 "Hot Squeeze Put on Tough Alloys," p. 67, Steel, March 9, 1953.  
 "Titanium Metal and Its Future," 1st par. p. 32, Harvard Business School, Cambridge, Mass., March 3, 1952.  
 60 "The Extrusion of Titanium," by Alvin M. Sabroff et al., Battelle Memorial Institute, WADC Tech. Report 54-555, March 1955.